# EUROPEAN PATENT SPECIFICATION

(11) **EP 4 035 903 B1**
(45) Date of publication and mention of the grant of the patent: **01.11.2023**
(21) Application number: 20868863.0
(22) Date of filing: 16.09.2020
(51) Int. Cl.: B42D 25/324, B42D 25/328, B42D 25/351, B42D 25/373, B42D 25/425, B42D 25/445

(54) **MULTILAYER BODY OPTICAL ANTI-COUNTERFEITING ELEMENT AND MANUFACTURING METHOD THEREFOR**
OPTISCHES FÄLSCHUNGSSCHUTZELEMENT MIT MEHRLAGIGEM KÖRPER UND HERSTELLUNGSVERFAHREN DAFÜR
ÉLÉMENT ANTI-CONTREFAÇON OPTIQUE À CORPS MULTICOUCHE ET SON PROCÉDÉ DE FABRICATION

(30) Priority: 29.09.2019 CN 201910932440
(43) Date of publication of application: 03.08.2022
(73) Proprietor: Zhongchao Special Security Technology Co., Ltd, Beijing 100070 (CN); China Banknote Printing and Minting Corp., Beijing 100044 (CN)
(72) Inventor: HU, Chunhua, Beijing 100070 (CN); SUN, Kai, Beijing 100070 (CN); ZHANG, Baoli, Beijing 100070 (CN); ZHU, Jun, Beijing 100070 (CN)
(74) Representative: Glawe, Delfs, Moll
(86) International application number: PCT/CN2020/115557
(87) International publication number: WO 2021/057574

(56) References cited:
- EP-A1- 3 208 099
- EP-B1- 1 182 054
- CN-A- 104 647 938
- CN-A- 105 015 215
- CN-A- 106 891 637
- CN-A- 107 405 942
- CN-A- 109 895 527
- DE-A1-102015 010 744

## Description

### Technical Field

The disclosure relates to the technical field of optical anti-counterfeiting technology, and in particular to an optical anti-counterfeiting element and a manufacturing method for an optical anti-counterfeiting element.

### Background

In order to prevent counterfeits produced by scanning and copying, the optical anti-counterfeiting technology is widely used in various high safety or high value-added printed materials such as banknotes, credit cards, passports, securities and product packaging, and has achieved extremely excellent effects.

In various optical anti-counterfeiting technologies, optical effects forming by the microstructure include diffraction, non-diffraction, etc., which is widely used by high brightness and obvious dynamic effect. The microstructure optical anti-counterfeiting technology generally uses a metal reflecting layer, for example aluminum, so as to increase the brightness of the image. Wherein, the holographic technology, the most widely used optical anti-counterfeiting technology in optical films at present, is developed by utilizing the diffraction effect formed by the microstructure, and has been used in anti-counterfeiting lines of 5 yuan, 10 yuan, 20 yuan, 50 yuan and 100 yuan in the fifth set of 1999 edition of RMB. In addition, the multilayer functional coating group technology has strong optical discoloration effect under different observation angles, or obvious discoloration effect under reflection and transmission observation, thereby drawing increasing attention from people, and is generally known as the multilayer interference optical variation technology. The classical multilayer interference coating generally uses the sandwich type Fabry-Perot interference cavity structure formed by a reflecting layer, a dielectric layer and an absorbing layer. The reflecting layer is generally made of high-brightness metal materials, the dielectric layer is generally made of transparent inorganic or organic materials, and the absorbing layer, also known as a semitransparent layer, is generally made of thin metal materials having excellent absorption. The security line of 100 yuan in the fifth set of 2015 edition of RMB uses the multilayer interference optical variation technology, which is magenta under front observation and green under inclined observation.

If the characteristics of the optical microstructure, the high-brightness metal reflecting layer and the multilayer functional coating group are integrated into the same optical anti-counterfeiting element, the optical anti-counterfeiting effect will be greatly enhanced. Patent application CN 200980104829.3 provided the preparation of the optical anti-counterfeiting product integrating the multilayer interference optically variable coating and the high-brightness metal reflecting layer by means of a local printing and hollowing process, that is, some regions have multilayer interference optically variable characteristics, some regions have optical characteristics of the high-brightness metal reflecting layer, and further, the other regions have the perspective hollow effect. However, the mutual alignment accuracy of the three regions in the patent application depends on the printing accuracy, which is generally above 100µm, resulting in limitations on the application in high-end anti-counterfeiting optical products to a certain extent.

Document CN 106891637 A discloses an optical anti-counterfeiting element having a first microstructure and a second microstructure.

Therefore, it is of great significance to manufacture optical anti-counterfeiting elements having characteristics of high-brightness metal reflecting layer and multilayer interference optically variable characteristics and having zero positioning error between two characteristic regions. Further, if the optical anti-counterfeiting element further integrates the hollow characteristic, and the hollow region and the image region are also positioned with zero error, the anti-counterfeiting performance of the product will be further improved.

### Summary

The objective of the disclosure is to provide a multilayer body optical anti-counterfeiting element and a manufacturing method therefor. During observation from a first side and/or a second side of the optical anti-counterfeiting element, the optical anti-counterfeiting element has a characteristic of a high-brightness metal reflecting layer and a characteristic of a multilayer functional coating group (especially an interference optically variable coating) at the same time, such that a product having the optical anti-counterfeiting element has excellent comprehensive integrated anti-counterfeiting performance. Further, if the optical anti-counterfeiting element further integrates a hollow characteristic, and a hollow region and an image region are positioned with zero error, the anti-counterfeiting performance of the product may be further improved.

In order to achieve the above objective, the present invention provides an optical anti-counterfeiting element as defined in claim 1.

Since the two image regions (the first region and the second region) presented by reflection observation are determined by the microstructure, thereby having a zero positioning error characteristic.

A specific volume of a relief structure mentioned herein refers to a ratio of an assumed liquid volume of just completely covering a surface of the relief structure to a projection area of the relief structure on the horizontal plane under the condition that the relief structure is placed in a horizontal state; the disclosure further relates to another important physical quantity, i.e. a depth-to-width ratio of the relief structure, which refers to a ratio of a depth of the relief structure to a width (or a period of a periodic structure) of the relief structure; according to this definition, the depth-to-width ratio is a dimensionless physical quantity, and a dimension of the specific volume is µm³/µm²; according to this definition, a flat structure is regarded as the relief structure having zero depth-to-width ratio and zero specific volume; the depth-to-width ratio and the specific volume are two physical quantities which have no direct relation in quantity; for example, if a structure A is a one-dimensional sawtooth grating having a depth of 1µm and a period of 1µm, a depth-to-width ratio of the structure A is 1, and a specific volume of the structure A is 0.5µm³/µm²; if a structure B is a one-dimensional sawtooth grating having a depth of 2µm and a period of 4µm, a depth-to-width ratio of the structure B is 0.5, and a specific volume of structure B is 1µm³/µm²; that is, the depth-to-width ratio of the structure A is greater than the depth-to-width ratio of the structure B, and the specific volume of the structure B is greater than the specific volume of the structure A; a difference of the specific volumes of the first microstructure and the second microstructure is a basis for removing a second coating in the second region; and a coating on a particular microstructure is accurately removed on the basis of the difference of the specific volume, which will be further described in the Detailed Description of the Embodiments.

Generally, the first microstructure or the second microstructure is a periodic structure or one structure or a combined structure in the periodic structure; and a cross-sectional structure of the first microstructure or the second microstructure is any one structure or a combined structure formed by at least any two structures of a sinusoidal structure, a rectangular grating structure, a trapezoidal grating structure, a blazed grating structure and an arc-shaped grating structure.

In an implementation mode, the specific volume of the first microstructure is greater than or equal to 0µm³/µm² and less than 0.5µm³/µm²; and the specific volume of the second microstructure is greater than 0.4µm³/µm² and less than 3µm³/µm².

In an implementation mode, the first coating is adjacently connected to the relief structure layer.

In an implementation mode, a material of the first coating or the second coating is any one metal or an alloy formed by combining at least any two metals of nickel, chromium, aluminum, silver, copper, tin and titanium; and a material of the dielectric layer is any one compound or a mixture formed by at least any two compounds of magnesium fluoride, silicon dioxide, zinc sulfide, titanium nitride, titanium dioxide, titanium monoxide, titanium sesquioxide, trititanium pentoxide, tantalum pentoxide, niobium pentoxide, cerium dioxide, bismuth trioxide, chromium oxide green, iron oxide, hafnium oxide and zinc oxide.

In an implementation mode, the functional coating group is a multilayer interference optically variable coating, and the optical anti-counterfeiting element on any side of the multilayer interference optically variable coating has an interference optically variable characteristic.

Further, in order to make the product capable of having an accurate positioning hollow characteristic, the relief structure layer further includes a third region having a third microstructure, a depth-to-width ratio of the third microstructure is greater than a depth-to-width ratio of the second microstructure, and a specific volume of the third microstructure is greater than a specific volume of the first microstructure; the first coating and the second coating are not located in the third region; and the optical anti-counterfeiting element has a hollow characteristic in the third region. A difference of the specific volumes of the third microstructure and the first microstructure and a difference of a depth-to-width ratios of the third microstructure and the second microstructure are a basis for removing both of the first coating and the second coating in the third region. A coating on a particular microstructure is accurately removed on the basis of the difference of the depth-to-width ratio, which will be further described in the Detailed Description of the Embodiments. In an implementation mode, the depth-to-width ratio of the third microstructure is greater than 0.2 and less than 1; the depth-to-width ratio of the second microstructure is greater than 0 and less than 0.3; and the specific volume of third microstructure is greater than 0.4µm³/µm² and less than 3µm³/µm².

The invention further provides a manufacturing method for an optical anti-counterfeiting element as defined in claim 9.

In an implementation mode, the relief structure layer in S1) further includes a third region having a third microstructure, a depth-to-width ratio of the third microstructure is greater than a depth-to-width ratio of the second microstructure, and a specific volume of the third microstructure is greater than a specific volume of the first microstructure.

In an implementation mode, the manufacturing method further includes: S4) placing a semi-finished product in S3) into an atmosphere capable of reacting with the first coating until part or all of the first coating and the second coating which are located in the third region are removed.

In an implementation mode, the first coating or the second coating in S3) includes an aluminum layer, or the first coating and the second coating in S3) include an aluminum layer; and
an acid liquor or an alkali liquor is selected as the atmosphere capable of reacting with the second coating in S3); an acid liquor or an alkali liquor is selected as the atmosphere capable of reacting with the first coating in S4).

In an implementation mode, the manufacturing method further includes: applying an inorganic or organic coating or a painting layer process to achieve other optical anti-counterfeiting functions or auxiliary functions.

Other features and advantages of the embodiment of the disclosure will be described in detail in the Brief Description of the Drawings that follows.

### Brief Description of the Drawings

The drawings, which are used for providing further understanding of the embodiment of the disclosure and constitute a part of the description, together with the following particular implementation, serve to explain the embodiment of the disclosure instead of limiting same. In the drawings:
Fig. 1 shows a top view of a first exemplary optical anti-counterfeiting element of the embodiment of the disclosure;
Fig. 2 shows a possible cross-sectional view of the first exemplary optical anti-counterfeiting element in an X-X direction of the embodiment of the disclosure;
Fig. 3 shows a cutaway view of an exemplary element after formation of a relief structure layer in a process of manufacturing the first exemplary optical anti-counterfeiting element of the embodiment of the disclosure;
Fig. 4 shows a cutaway view of the exemplary element after formation of a functional coating group in the process of manufacturing the first exemplary optical anti-counterfeiting element of the embodiment of the disclosure;
Fig. 5 shows a cutaway view of the exemplary element after formation of a protective layer in the process of manufacturing the first exemplary optical anti-counterfeiting element of the embodiment of the disclosure;
Fig. 6 shows a cutaway view of the exemplary element after a corrosion atmosphere in the process of manufacturing the first exemplary optical anti-counterfeiting element of the embodiment of the disclosure;
Fig. 7 shows a top view of a second exemplary optical anti-counterfeiting element of the embodiment of the disclosure;
Fig. 8 shows a possible cross-sectional view of the second exemplary optical anti-counterfeiting element in an X-X direction of the embodiment of the disclosure;
Fig. 9 shows a cutaway view of an exemplary element after formation of a relief structure layer in a process of manufacturing the second exemplary optical anti-counterfeiting element of the embodiment of the disclosure;
Fig. 10 shows a cutaway view of the exemplary element after formation of a functional coating group in the process of manufacturing the second exemplary optical anti-counterfeiting element of the embodiment of the disclosure;
Fig. 11 shows a cutaway view of the exemplary element after formation of a protective layer in the process of manufacturing the second exemplary optical anti-counterfeiting element of the embodiment of the disclosure; and
Fig. 12 shows a cutaway view of the exemplary element after a corrosion atmosphere in the process of manufacturing the second exemplary optical anti-counterfeiting element of the embodiment of the disclosure.

### Description of reference numerals:

| | | | |
|---|---|---|---|
| 1. | a substrate | 2. | a relief structure layer |
| 31. | a first coating | 32. | a dielectric layer |
| 33. | a second coating | 3. | a functional coating group |
| 4. | a protective layer | | |
| 5. | an other functional coating | | |

### Detailed Description of the Embodiments

The particular implementation of the embodiment of the disclosure is described in detail below in conjunction with the drawings. It should be understood that the particular implementation described herein is merely illustrative of the embodiment of the disclosure and is not intended to limit the embodiment of the disclosure.

### Embodiment 1

As shown in Fig. 1, an optical anti-counterfeiting element includes a first region A and a second region B, wherein the first region A has a combined optical characteristic of a first optical microstructure and a functional coating group, and the second region B has a combined optical characteristic of a second optical microstructure and a first coating. The two regions are strictly positioned to each other. Partial lines of an image may be very fine. For example, the partial lines are less than 50µm. In an embodiment, the functional coating group is a multilayer interference optically variable coating, and a first coating is a metal reflection coating (e.g. an aluminum layer), such that the first region A appears an interference optically variable characteristic and the second region B appears a characteristic of the common metal reflection coating.

As shown in Fig. 2, the optical anti-counterfeiting element includes a substrate 1, a relief structure layer 2, a first coating 31, a dielectric layer 32, a second coating 33, a protective layer 4 and an other functional coating 5, wherein the first coating 31, the dielectric layer 32 and the second coating 33 form a functional coating group 3; the substrate 1 and the relief structure layer 2 is usually composed of a transparent material; the relief structure layer 2 includes the first region A composed of a first microstructure and the second region B composed of a second microstructure, a specific volume of the second microstructure is greater than a specific volume of the first microstructure; the functional coating group 3 composed of the first coating 31, the dielectric layer 32 and the second coating 33 is arranged on the first region A, and the first coating 31 and the dielectric layer 32 are arranged on the second region B. Usually, the dielectric layer 32 is a colorless transparent material and does not provide special optical effects in the second region B. During observation from above and/or below the anti-counterfeiting element, the first region A appears a combined optical characteristic of the first microstructure and the functional coating group 3, and the second region B appears a combined optical characteristic of the second microstructure and the first coating 31. If the first coating 31 is semitransparent and the second coating 33 is non-transparent or substantially non-transparent, the optical anti-counterfeiting element must be observed from below; if the first coating 31 is non-transparent or substantially non-transparent and the second coating 33 is semitransparent, the optical anti-counterfeiting element must be observed from above; and if both the first coating 31 and the second coating 33 are semitransparent, the optical anti-counterfeiting element may be observed both from below or above. The functional coating group 3 is adjacently connected to a protective layer 4. The protective layer 4 is a natural product in a manufacturing process and generally does not provide additional optical effects. Particularly, in the first region A, the first coating 31, the dielectric layer 32 and the second coating 33 are used as a reflecting layer, a dielectric layer and an absorbing layer respectively and are combined to form a multilayer interference optically variable coating, that is, the first region A has a combined anti-counterfeiting characteristic of the first microstructure and the multilayer interference optically variable coating; and the second region B has a combined anti-counterfeiting characteristic of the second microstructure and a traditional reflecting layer. The other functional coating 5 may be provided as required, such as a bonding layer that has a function of bonding a protected main product.

A method for preparing an optical anti-counterfeiting element as shown in Fig. 2 according to the disclosure is described below in conjunction with Figs. 3-6. The method includes S1-S4. For simplicity of description, a multilayer interference optically variable coating is selected as the functional coating group 3, and the first coating 31, the dielectric layer 32 and the second coating 33 are used as a reflecting layer, a dielectric layer and an absorbing layer respectively.

S1, forming the relief structure layer 2 on a first side of the substrate 1, wherein the relief structure layer 2 at least includes the first region A composed of the first microstructure and the second region B composed of the second microstructure, a specific volume of the second microstructure is greater than a specific volume of the first microstructure, which is as shown in Fig. 3.

The substrate 1 may be at least locally transparent, or a colorless dielectric layer, or a transparent medium film having a functional coating layer on a surface, or a multilayer film formed through compounding. The substrate 1 is generally formed by a film material having excellent physical and chemical resistance and high mechanical strength, for example, a plastic film of a polyethylene terephthalate (PET) film, a polyethylene terephthalate (PEN) film, a polypropylene (PP) film, etc. may be used to form the substrate 1. In an embodiment, the substrate 1 is formed by the PET material. A bonding enhancement layer may be included on the substrate 1 to enhance bonding of the substrate 1 to the relief structure layer 2. A stripping layer may also be included on the substrate 1 to achieve separation of the substrate 1 in the final product from the relief structure layer 2.

The relief structure layer 2 may be formed by performing batch copying by means of processing manners of ultraviolet casting, mold pressing, nano-imprinting, etc. For example, the relief structure layer 2 may be formed by a thermoplastic resin by means of a mold pressing process, that is, the thermoplastic resin coating on the substrate 1 in advance is heated to be softened and deformed when passing through a high-temperature metal template, such that a specific relief structure is formed, and then is cooled and molded. The relief structure layer 2 may also be formed by a radiation curing casting process, that is, the substrate 1 is coated with a radiation curing resin, irradiating the substrate 1 by radiation of ultraviolet light, an electron beam, etc. while pushing and pressing a master plate on the substrate 1, so as to cure the above materials, and then the master plate is removed, thereby forming the relief structure layer 2.

In order to satisfy a requirement of subsequent coating removal, the specific volume of the second microstructure is greater than the specific volume of the first microstructure. In an embodiment, the specific volume of the first microstructure is greater than or equal to 0µm³/µm² and less than 0.5µm³/µm²; and the specific volume of the second microstructure is greater than 0.4µm³/µm² and less than 3µm³/µm².

The first microstructure or the second microstructure is one structure or a combined structure of a periodic structure and a non-periodic structure; and a cross-sectional structure of the first microstructure or the second microstructure is any one structure or a combined structure formed by at least any two structures of a sinusoidal structure, a rectangular grating structure, a trapezoidal grating structure, a blazed grating structure and an arc-shaped grating structure. Size and horizontal arrangement of the first microstructure and the second microstructure are determined by a required optical effect. A flat structure may be selected as the first microstructure.

S2) forming the functional coating group 3 composed of the first coating 31, the dielectric layer 32 and the second coating 33 on the relief structure layer 2, which is as shown in Fig. 4.

In the embodiment, the multilayer interference optically variable coating is selected as the functional coating group 3, the first coating 31, the dielectric layer 32 and the second coating 33 are used as the reflecting layer, the dielectric layer and the absorbing layer respectively, that is, the first coating 31 is non-transparent or basically non-transparent, and the second coating 33 is semitransparent.

The first coating 31 serves as the reflecting layer in the interference optically variable coating. A material of the first coating 31 may be any one metal or a mixture or an alloy of at least any two metals of Al, Cu, Ni, Cr, Ag, Fe, Sn, Au and Pt. A thickness of the first coating 31 is generally selected to be greater than 10nm and less than 80nm, more specifically, greater than 20nm and less than 50nm. If a metal reflection coating is too thin, brightness is not enough; and if the metal reflection coating is too thick, fastness of the metal reflection coating and the relief structure layer 2 is poor, and cost is increased. The first coating 31 may generally be formed on the relief structure layer 2 by means of physical and/or chemical vapor deposition methods, such as, but not limited to, thermal evaporation, magnetron sputtering, metal organic chemical vapor deposition (MOCVD), etc. In an embodiment, the first coating 31 is formed on the relief structure layer 2 in a homomorphic coverage manner with a uniform surface density.

The dielectric layer 32 provides a function of a dielectric layer in a Fabry-Perot interference cavity. The dielectric layer 32 is generally formed by means of a vapor deposition method, and a material of the dielectric layer may be selected from MgF₂, Sn, Cr, ZnS, ZnO, TiO₂, MgO, SiO₂, or a mixture thereof. After vapor deposition, a surface topography of the dielectric layer 32 and a topography of the first coating 31 are homomorphic or substantially homomorphic. A thickness of the dielectric layer 32 is determined by an effect required by the final interference optically variable coating and is generally greater than 100nm and less than 600nm.

The second coating 33 serves as the absorbing layer in the interference optically variable coating. The absorbing layer is generally made of a thin metal material, and appears a semitransparent characteristic in light transmission. The second coating 33 may be composed of any one metal or an alloy of at least two metals of aluminum, silver, copper, tin, chromium, nickel and titanium. In an embodiment, aluminum is selected since aluminum has low cost and easy to remove by an acid liquor or an alkali liquor. The second coating 33 is generally formed by means of a vapor deposition method. After vapor deposition, a surface topography of the second coating 33 and a topography of the first coating 31 and the dielectric layer 32 are homomorphic or substantially homomorphic. A thickness of the second coating 33 is generally greater than 2nm and less than 10nm.

S3, forming a protective layer 4 on the functional coating group 3, which is as shown in Fig. 5.

The protective layer 4 is generally formed by means of a printing process. The specific volume of the first microstructure on the relief structure layer 2 is less than the specific volume of the second microstructure, and the functional coating group 3 is generally formed on the relief structure layer 2 in a homomorphic coverage manner, and therefore, a specific volume of a microstructure on a surface of the functional coating group 3 in the first region A is still less than a specific volume of a microstructure on a surface of the functional coating group 3 in the second region B. A proper printing amount of the protective layer 4 may be selected, such that a minimum thickness of the protective layer 4 at the microstructure of the surface of the functional coating group 3 in the first region A is obviously greater than a minimum thickness of the protective layer 4 at the microstructure of the surface of the functional coating group 3 in the second region B. A minimum thickness of the protective layer 4 at the microstructure is generally located at the topmost of the microstructure. Therefore, a protective function of the protective layer 4 for the functional coating group 3 in the first region A is obviously higher than a protective function of the protective layer 4 for the functional coating group 3 in the second region B. Coating weight of the protective layer 4 per unit area is generally required to be greater than 0.1 g/m² and less than 1 g/m². The smaller viscosity before coating of the protective layer 4, the more beneficial leveling is, and therefore, viscosity of a protective glue solution is generally less than 100cP, more specifically, less than 50cP. A composition of the protective layer 4 may be any one of polyester, polyurethane and acrylic resin, or varnish or ink by combining at least any two thereof as a main resin.

S4, placing a multilayer structure body in S3 into an atmosphere capable of reacting with the material of the second coating 33 until part or all of the second coating located in the second region B are removed, which is as shown in Fig. 6.

As mentioned above, the protective function of the protective layer 4 on the functional coating group 3 in the first region A is obviously higher than the protective function of the protective layer 4 on the functional coating group 3 in the second region B. Therefore, within a certain period of time, a corrosion atmosphere will reach and corrode the second coating 33 by means of a vulnerable point of the protective layer 4 in the second region B; and within the time, the protective layer 4 effectively protects the second coating 33 in the first region A. Generally, the dielectric layer 32 does not act with the corrosion atmosphere, that is, the dielectric layer 32 may effectively protect the first coating 31. Thus, the functional coating group 3 accurately located in the first region A and the first coating 31 accurately located in the second region B are acquired. If the second coating 33 is aluminum or a coating including aluminum, the corrosion atmosphere may be an acid liquor or an alkali liquor. Usually, after the second coating on the second region B is corroded, the protective layer on the coating floats along therewith. Sometimes, after the second coating on the second region B is corroded, the protective layer on the coating may partially or even completely remain on the multilayer body, which does not influence implementation of subsequent processes.

Hereto, a semi-finished product of optical anti-counterfeiting element having the optical characteristic appeared by the functional coating group 3 in the first region A and the optical characteristic appeared by the first coating 31 in the second region B is acquired.

The method for manufacturing an optical anti-counterfeiting element shown in Fig. 2 generally further includes: after S4, applying the other functional coating 5, such as anti-aging glue, to protect an optical coating, and/or hot melt glue, to bond same to other substrates.

### Embodiment 2

As shown in Fig. 7, an optical anti-counterfeiting element includes a first region A, a second region B and a third region C, wherein the first region A has a combined optical characteristic of a first optical microstructure and a functional coating group, the second region B has a combined optical characteristic of a second optical microstructure and a first coating, and the third region has a hollow characteristic under perspective observation. The third regions are strictly positioned to each other. For example, the third region C shown in Fig. 7 is strictly located at a boundary of the second region B. An image or hollow lines may be very fine frequently. For example, the image or the hollow lines are less than 50µm. In an embodiment, the functional coating group is a multilayer interference optically variable coating, and a first coating is a metal reflection coating (e.g. an aluminum layer), such that the first region A appears an interference optically variable characteristic and the second region B appears a characteristic of the common metal reflection coating.

As shown in Fig. 8, the optical anti-counterfeiting element includes a substrate 1, a relief structure layer 2, a first coating 31, a dielectric layer 32, a second coating 33, a protective layer 4 and an other functional coating 5, wherein the first coating 31, the dielectric layer 32 and the second coating 33 form a functional coating group 3. The substrate 1 and the relief structure layer 2 is usually composed of a transparent material; the relief structure layer 2 includes a first region A composed of a first microstructure, a second region B composed of a second microstructure and a third region C composed of a third microstructure, a specific volume of the second microstructure is greater than a specific volume of the first microstructure, a specific volume of the third microstructure is greater than a specific volume of the first microstructure, and a depth-to-width ratio of the third microstructure is greater than a depth-to-width ratio of the second microstructure. The functional coating group 3 composed of the first coating 31, the dielectric layer 32 and the second coating 33 is arranged on the first region A, the first coating 31 and the dielectric layer 32 are arranged on the second region B, and the first coating 31 and the second coating 33 are not arranged on the third region C. Usually, the dielectric layer 32 is a colorless transparent material and does not provide special optical effects in the second region B. During observation from above and/or below the optical anti-counterfeiting element, the first region A appears a combined optical characteristic of the first microstructure and the functional coating group 3, and the second region B appears a combined optical characteristic of the second microstructure and the first coating 31. Since the first coating 31 and the second coating 33 are not arranged, when the optical anti-counterfeiting element is observed through transmission, the third region C has a hollow characteristic. The functional coating group 3 is adjacently connected to a protective layer 4. The protective layer 4 is a natural product in a manufacturing process and generally does not provide additional optical effects. Particularly, in the first region A, the first coating 31, the dielectric layer 32 and the second coating 33 are formed into a multilayer interference optically variable coating as a reflecting layer, a dielectric layer and an absorbing layer respectively, that is, the first region A has a combined anti-counterfeiting characteristic of the first microstructure and the multilayer interference optically variable coating; and the second region B has a combined anti-counterfeiting characteristic of the second microstructure and the common reflecting layer. The other functional coating 5 may be provided as required, such as a bonding layer that has a function of bonding a protected main product.

A method for preparing an optical anti-counterfeiting element as shown in Fig. 7 according to the disclosure is described below in conjunction with Figs. 9-12. The method includes S1'-S4'. For simplicity of description, a multilayer interference optically variable coating is selected as the functional coating group 3, and the first coating 31, the dielectric layer 32 and the second coating 33 are used as a reflecting layer, a dielectric layer and an absorbing layer respectively.

S1', forming a relief structure layer 2 on a first side of a substrate 1, wherein the relief structure layer 2 includes the first region A composed of the first microstructure, the second region B composed of the second microstructure and the third region C composed of the third microstructure, a specific volume of the second microstructure is greater than a specific volume of the first microstructure, a specific volume of the third microstructure is greater than a specific volume of the first microstructure, and a depth-to-width ratio of the third microstructure is greater than a depth-to-width ratio of the second microstructure, which is as shown in Fig. 9.

The substrate 1 may be at least locally transparent, or a colorless dielectric layer, or a transparent medium film having a functional coating layer on a surface, or a multilayer film formed through compounding. The substrate 1 is generally formed by a film material having excellent physical and chemical resistance and high mechanical strength, for example, a plastic film of a polyethylene terephthalate (PET) film, a polyethylene terephthalate (PEN) film, a polypropylene (PP) film, etc. may be used to form the substrate 1. In an embodiment, the substrate 1 is formed by the PET material. A bonding enhancement layer may be included on the substrate 1 to enhance bonding of the substrate 1 to the relief structure layer 2. A stripping layer may also be included on the substrate 1 to achieve separation of the substrate 1 in the final product from the relief structure layer 2.

The relief structure layer 2 may be formed by performing batch copying by means of processing manners of ultraviolet casting, mold pressing, nano-imprinting, etc. For example, the relief structure layer 2 may be formed by a thermoplastic resin by means of a mold pressing process, that is, the thermoplastic resin coating on the substrate 1 in advance is heated to be softened and deformed when passing through a high-temperature metal template, such that a specific relief structure is formed, and then is cooled and molded. The relief structure layer 2 may also be formed by a radiation curing casting process, that is, the substrate 1 is coated with a radiation curing resin, irradiating the substrate 1 by radiation of ultraviolet light, an electron beam, etc. while pushing and pressing a master plate on the substrate, so as to cure the above materials, and then the master plate is removed, thereby forming the relief structure layer 2.

In order to satisfy a requirement of subsequent coating removal, the specific volume of the second microstructure is greater than the specific volume of the first microstructure, the specific volume of the third microstructure is greater than the specific volume of the first microstructure, and the depth-to-width ratio of the third microstructure is greater than the depth-to-width ratio of the second microstructure. In an embodiment, the specific volume of the first microstructure is greater than or equal to 0µm³/µm² and less than 0.5µm³/µm², the specific volume of the second microstructure is greater than 0.4µm³/µm² and less than 3µm³/µm², and the specific volume of third microstructure is greater than 0.4µm³/µm² and less than 3µm³/µm²; and the depth-to-width ratio of the second microstructure is greater than 0 and less than 0.3, and the depth-to-width ratio of the third microstructure is greater than 0.2 and less than 1. The depth-to-width ratio of the first microstructure is not limited, and may be configured according to a required optical effect.

The first microstructure, the second microstructure or the third microstructure is one structure or a combined structure of a periodic structure and a non-periodic structure; and a cross-sectional structure of the first microstructure, the second microstructure or the third microstructure is any one structure or a combined structure formed by at least any two structures of a sinusoidal structure, a rectangular grating structure, a trapezoidal grating structure, a blazed grating structure and an arc-shaped grating structure. Size and horizontal arrangement of the first microstructure and the second microstructure are determined by a required optical effect. A flat structure may be selected as the first microstructure. The third microstructure is only used for hollowing and generally does not provide additional optical effects, and therefore, may be simplified, such as a blazed grating which is arranged in one dimension and has a cross-sectional of an isosceles triangle having a bottom edge width of 10µm and a height of 5µm (i.e., a depth-to-width ratio of 0.5 and a specific volume of 2.5 µm³/µm²).

S2', forming the functional coating group 3 composed of the first coating 31, the dielectric layer 32 and the second coating 33 on the relief structure layer 2, which is as shown in Fig. 10.

In the embodiment, the multilayer interference optically variable coating is selected as the functional coating group 3, the first coating 31, the dielectric layer 32 and the second coating 33 are used as the reflecting layer, the dielectric layer and the absorbing layer respectively, that is, the first coating 31 is non-transparent or basically non-transparent, and the second coating 33 is semitransparent.

The first coating 31 serves as the reflecting layer in the interference optically variable coating. A material of the first coating 31 may be any one metal or a mixture or an alloy of at least any two metals of Al, Cu, Ni, Cr, Ag, Fe, Sn, Au and Pt. In an embodiment, aluminum is selected since aluminum has low cost and easy to remove by an acid liquor or an alkali liquor. A thickness of the first coating 31 is generally selected to be greater than 10nm and less than 80nm, more specifically, greater than 20nm and less than 50nm. If the metal reflection coating is too thin, brightness is not enough; and if the metal reflection coating is too thick, fastness of the metal reflection coating and the relief structure layer 2 is poor, and cost is increased. The first coating 31 may generally be formed on the relief structure layer 2 by means of physical and/or chemical vapor deposition methods, such as, but not limited to, thermal evaporation, magnetron sputtering, MOCVD, etc. In an embodiment, the first coating 31 is formed on the relief structure layer 2 in a homomorphic coverage manner with a uniform surface density.

The dielectric layer 32 provides a function of a dielectric layer in a Fabry-Perot interference cavity. The dielectric layer 32 is generally formed by means of a vapor deposition method, and a material of the dielectric layer may be selected from MgF₂, Sn, Cr, ZnS, ZnO, TiO₂, MgO, SiO₂, or a mixture thereof. After vapor deposition, a surface topography of the dielectric layer 32 and a topography of the first coating 31 are homomorphic or substantially homomorphic. A thickness of the dielectric layer 32 is determined by an effect required by the final interference optically variable coating and is generally greater than 100nm and less than 600nm.

The second coating 33 serves as the absorbing layer in the interference optically variable coating. The absorbing layer is generally made of a thin metal material, and appears a semitransparent characteristic in light transmission. The second coating 33 may be composed of any one metal or an alloy of at least two metals of aluminum, silver, copper, tin, chromium, nickel and titanium. In an embodiment, aluminum is selected since aluminum has low cost and easy to remove by an acid liquor or an alkali liquor. The second coating 33 is generally formed by means of a vapor deposition method. After vapor deposition, a surface topography of the second coating 33 and a topography of the first coating 31 and the dielectric layer 32 are homomorphic or substantially homomorphic. A thickness of the second coating 33 is generally greater than 2nm and less than 10nm.

S3', forming a protective layer 4 on the functional coating group 3, which is as shown in Fig. 11.

The protective layer 4 is generally formed by means of a printing process. The specific volume of the first microstructure on the relief structure layer 2 is less than the specific volumes of the second microstructure and the third microstructure, and the functional coating group 3 is generally formed on the relief structure layer 2 in a homomorphic coverage manner, and therefore, a specific volume of a microstructure on a surface of the functional coating group 3 in the first region A is still less than specific volumes of microstructures on a surface of the functional coating group 3 in the second region B and the third region C. A proper printing amount of the protective layer 4 may be selected, such that a minimum thickness of the protective layer 4 at the microstructure of the surface of the functional coating group 3 of the protective layer 4 in the first region A is obviously greater than a minimum thickness of the protective layer 4 at the microstructure of the surface of the functional coating group 3 in the second region B and the third region C. A minimum thickness of the protective layer 4 at the microstructure is generally located at the topmost of the microstructure. Thus, a protective function of the protective layer 4 for the functional coating group 3 in the first region A is obviously higher than a protective function of the protective layer 4 for the functional coating group 3 in the second region B and the third region C. Coating weight of the protective layer 4 per unit area is generally required to be greater than 0.1 g/m² and less than 1g/m². The smaller viscosity before coating of the protective layer 4, the more beneficial leveling is, and therefore, viscosity of a protective glue solution is generally less than 100cP, more specifically, less than 50cP. A composition of the protective layer 4 may be any one of polyester, polyurethane and acrylic resin, or varnish or ink by combining at least any two thereof as a main resin.

S4', placing a multilayer structure body in S3' into an atmosphere capable of reacting with materials of the first coating 31 and the second coating 33 until part or all of the second coating located in the second region B and the first coating and the second coating located in the third region C are removed, which is as shown in Fig. 12.

As mentioned above, the protective function of the protective layer 4 on the functional coating group 3 in the first region A is obviously higher than the protective function of the protective layer 4 on the functional coating group 3 in the second region B and the third region C. Therefore, within a certain period of time, a corrosion atmosphere will reach and corrode the second coating 33 by means of a vulnerable point of the protective layer 4 in the second region B and the third region C; and since the depth-to-width ratio of the third microstructure is greater than the depth-to-width ratio of the second microstructure, more cracks are formed in the dielectric layer 32 in the third region C than the dielectric layer 32 in the second region B, and therefore, a protective function of the dielectric layer 32 in the third region C on the first coating beneath it is worse than a protective function of the dielectric layer 32 in the second region B on the first coating beneath it. Therefore, in the third region C, after corroding the second coating 33 in the third region C, the corrosion atmosphere continues corroding the first coating 31 by means of the vulnerable point of the dielectric layer 32; and in the second region B, the first coating 31 is effectively protected by the dielectric layer 32 to be reserved. Thus, the functional coating group 3 accurately located in the first region A and the first coating 31 accurately located in the second region B are acquired; and the second coating located in the second region B and the functional coating group 3 located in the third region C are accurately removed. If the first coating 31 and the second coating 33 are aluminum or a coating including aluminum, the corrosion atmosphere may be an acid liquor or an alkali liquor. Usually, after the second coating on the second region B and the third region C is corroded, the protective layer on the coating floats along therewith. Sometimes, after the second coating on the second region B and the third region C is corroded, the protective layer on the coating may partially or even completely remain on a multilayer body, which does not influence implementation of subsequent working procedures.

Hereto, a semi-finished product of optical anti-counterfeiting element having the optical characteristic appeared by the functional coating group 3 in the first region A, the optical characteristic appeared by the first coating 31 in the second region B, and the hollow characteristic in the third region C is acquired.

The method for preparing an optical anti-counterfeiting element shown in Fig. 7 generally further includes: after S4', applying the other functional coating 5, such as anti-aging glue, to protect an optical coating, and/or hot melt glue, to bond same to other substrates.

The method for preparing an optical anti-counterfeiting element according to the disclosure is suitable for manufacturing windowing security lines, labels, marks, wide strips, transparent windows, coating films, etc. Anti-counterfeiting paper having a windowing security line is used for anti-counterfeiting of various high-safety products of banknotes, passports and securities.

The alternative implementation of the embodiment of the disclosure is described in detail above in conjunction with the drawings. However, the embodiment of the disclosure is not limited to specific details of the above embodiment. Within the scope of the technical concept of the embodiment of the disclosure, various simple modifications may be made to the technical solution of the embodiment of the disclosure, and these simple modifications all fall within the scope of protection of the embodiment of the disclosure.

It should also be noted that various specific technical characteristics described in the above particular implementation may be combined in any suitable manner, without contradiction. In order to avoid unnecessary repetition, the embodiment of the disclosure will not be described separately for various possible combinations.

Those skilled in the art may understand that all or part of steps in the methods of the above embodiments may be completed by instructing relevant hardware by means of a program, the program is stored in a storage medium and includes a plurality of instructions for making a single chip computer, a chip or a processor execute all or part of the steps of the methods of the various embodiments of the disclosure. The foregoing storage medium includes a universal serial bus (USB), a mobile hard disk, a read-only memory (ROM), a random access memory (RAM), a diskette or an optical disk, etc., which may store program codes.

In addition, various different implementations of the embodiment of the disclosure may also be combined randomly, so long as they fall within the scope of the claims.

## Claims

1. An optical anti-counterfeiting element, comprising:
a relief structure layer (2);
the relief structure layer (2) comprises a first region (A) having a first microstructure and a second region (B) having a second microstructure, a specific volume of the second microstructure is greater than a specific volume of the first microstructure;
a first coating (31), a dielectric layer (32), a second coating (33) and a protective layer (4) stacked in sequence are arranged on a side of the relief structure layer (2);
the first coating (31) and the dielectric layer (32) are located in the first region (A) and the second region (B), and the second coating (33) and the protective layer (4) are located in the first region (A) but not located in the second region (B); and
wherein, the first coating (31), the dielectric layer (32) and the second coating (33) form a functional coating group (3), the functional coating group (3) and the first microstructure have a combined optical characteristic in the first region (A), and the first coating (31) and the second microstructure have a combined optical characteristic in the second region (B).

2. The optical anti-counterfeiting element as claimed in claim 1, wherein
the first microstructure or the second microstructure is one structure or a combined structure of a periodic structure and a non-periodic structure; and
a cross-sectional structure of the first microstructure or the second microstructure is any one structure or a combined structure formed by at least any two structures of a sinusoidal structure, a rectangular grating structure, a trapezoidal grating structure, a blazed grating structure and an arc-shaped grating structure.

3. The optical anti-counterfeiting element as claimed in claim 1, wherein
the specific volume of the first microstructure is greater than or equal to 0µm³/µm² and less than 0.5µm³/µm²; and
the specific volume of the second microstructure is greater than 0.4µm³/µm² and less than 3µm³/µm².

4. The optical anti-counterfeiting element as claimed in claim 1, wherein
the first coating (31) is adjacently connected to the relief structure layer (2).

5. The optical anti-counterfeiting element as claimed in claim 1, wherein
a material of the first coating (31) or the second coating (33) is any one metal or an alloy formed by combining at least any two metals of nickel, chromium, aluminum, silver, copper, tin and titanium; and
a material of the dielectric layer (32) is any one compound or a mixture formed by at least any two compounds of magnesium fluoride, silicon dioxide, zinc sulfide, titanium nitride, titanium dioxide, titanium monoxide, titanium sesquioxide, trititanium pentoxide, tantalum pentoxide, niobium pentoxide, cerium dioxide, bismuth trioxide, chromium oxide green, iron oxide, hafnium oxide and zinc oxide.

6. The optical anti-counterfeiting element as claimed in claim 1, wherein
the functional coating group (3) is a multilayer interference optically variable coating, and the optical anti-counterfeiting element on any side of the multilayer interference optically variable coating has an interference optically variable characteristic.

7. The optical anti-counterfeiting element as claimed in claim 1, wherein
the relief structure layer (2) further comprises a third region (C) having a third microstructure, a depth-to-width ratio of the third microstructure is greater than a depth-to-width ratio of the second microstructure, and a specific volume of the third microstructure is greater than a specific volume of the first microstructure;
the first coating (31) and the second coating (33) are not located in the third region (C); and the optical anti-counterfeiting element has a hollow characteristic in the third region (C).

8. The optical anti-counterfeiting element as claimed in claim 7, wherein
the depth-to-width ratio of the third microstructure is greater than 0.2 and less than 1;
a depth-to-width ratio of the second microstructure is greater than 0 and less than 0.3; and
the specific volume of the third microstructure is greater than 0.4µm³/µm² and less than 3µm³/µm².

9. A manufacturing method for an optical anti-counterfeiting element, comprising:
S1) forming a relief structure layer (2), wherein the relief structure layer (2) comprises a first region (A) having a first microstructure and a second region (B) having a second microstructure, a specific volume of the second microstructure is greater than a specific volume of the first microstructure;
S2) forming a first coating, a dielectric layer, a second coating and a protective layer stacked in sequence on a side of the relief structure layer (2); and
S3) placing a semi-finished product in S2) into an atmosphere capable of reacting with the second coating until part or all of the second coating located in the second region (B) is removed, and at least reserving a first coating (31) and a second coating (33) stacked only in the first region (A), wherein the first coating (31) and the second coating (33) are non-removed parts of the first coating and the second coating which are located in the first region (A) respectively.

10. The manufacturing method for an optical anti-counterfeiting element as claimed in claim 9, wherein
the relief structure layer (2) in S1) further comprises a third region (C) having a third microstructure, a depth-to-width ratio of the third microstructure is greater than a depth-to-width ratio of the second microstructure, and a specific volume of the third microstructure is greater than a specific volume of the first microstructure.

11. The manufacturing method for an optical anti-counterfeiting element as claimed in claim 10, further comprising:
S4) placing a semi-finished product in S3) into an atmosphere capable of reacting with the first coating and the second coating until part or all of the first coating and the second coating which are located in the third region (C) are removed.

12. The manufacturing method for an optical anti-counterfeiting element as claimed in claim 11, wherein
the first coating (31) or the second coating (33) in S3) comprises an aluminum layer, or the first coating (31) and the second coating (33) in S3) comprise an aluminum layer; and
an acid liquor or an alkali liquor is selected as the atmosphere capable of reacting with the first coating and/or the second coating in S4).

13. The manufacturing method for an optical anti-counterfeiting element as claimed in any one of claims 9-12, further comprising:
applying an inorganic or organic coating or a painting layer process.

## Patentansprüche

1. Optisches Fälschungsschutzelement, umfassend:
eine Reliefstrukturschicht (2);
wobei die Reliefstrukturschicht (2) einen ersten Bereich (A) mit einer ersten Mikrostruktur und einen zweiten Bereich (B) mit einer zweiten Mikrostruktur umfasst, wobei ein spezifisches Volumen der zweiten Mikrostruktur größer als ein spezifisches Volumen der ersten Mikrostruktur ist;
eine erste Beschichtung (31), eine dielektrische Schicht (32), eine zweite Beschichtung (33) und eine Schutzschicht (4), die der Reihe nach gestapelt auf einer Seite der Reliefstrukturschicht (2) angeordnet sind;
wobei die erste Beschichtung (31) und die dielektrische Schicht (32) in dem ersten Bereich (A) und dem zweiten Bereich (B) angeordnet sind und die zweite Beschichtung (33) und die Schutzschicht (4) in dem ersten Bereich (A) angeordnet sind aber nicht in dem zweiten Bereich (B) angeordnet sind; und
wobei die erste Beschichtung (31), die dielektrische Schicht (32) und die zweite Beschichtung (33) eine funktionelle Beschichtungsgruppe (3) bilden, wobei die funktionelle Beschichtungsgruppe (3) und die erste Mikrostruktur eine kombinierte optische Charakteristik in dem ersten Bereich (A) aufweisen und die erste Beschichtung (31) und die zweite Mikrostruktur eine kombinierte optische Charakteristik in dem zweiten Bereich (B) aufweisen.

2. Optisches Fälschungsschutzelement gemäß Anspruch 1, wobei
die erste Mikrostruktur oder die zweite Mikrostruktur eine Struktur oder eine kombinierte Struktur einer periodischen Struktur und einer nichtperiodischen Struktur ist; und
eine Querschnittstruktur der ersten Mikrostruktur oder der zweiten Mikrostruktur eine beliebige Struktur von oder eine von wenigstens zwei beliebigen Strukturen von einer sinusartigen Struktur, einer rechteckigen Gitterstruktur, einer trapezartigen Gitterstruktur, einer Blazegitterstruktur und einer bogenförmigen Gitterstruktur gebildete kombinierte Struktur ist.

3. Optisches Fälschungsschutzelement gemäß Anspruch 1, wobei
das spezifische Volumen der ersten Mikrostruktur größer als oder gleich 0 µm³/µm² und kleiner als 0,5 µm³/µm² ist; und
das spezifische Volumen der zweiten Mikrostruktur größer als 0,4 µm³/µm² und kleiner als 3 µm³/µm² ist.

4. Optisches Fälschungsschutzelement gemäß Anspruch 1, wobei
die erste Beschichtung (31) mit der Reliefstrukturschicht (2) angrenzend verbunden ist.

5. Optisches Fälschungsschutzelement gemäß Anspruch 1, wobei
ein Material der ersten Beschichtung (31) oder der zweiten Beschichtung (33) ein beliebiges Metall von oder eine durch Kombinieren von wenigstens zwei beliebigen Metallen von Nickel, Chrom, Aluminium, Silber, Kupfer, Zinn und Titan gebildete Legierung ist; und
ein Material der dielektrischen Schicht (32) eine beliebige Verbindung von oder ein von wenigstens zwei beliebigen Verbindungen von Magnesiumfluorid, Siliciumdioxid, Zinksulfid, Titannitrid, Titandioxid, Titanmonoxid, Titansesquioxid, Trititanpentoxid, Tantalpentoxid, Niobpentoxid, Cerdioxid, Bismuttrioxid, Chromoxidgrün, Eisenoxid, Hafniumoxid und Zinkoxid gebildetes Gemisch ist.

6. Optisches Fälschungsschutzelement gemäß Anspruch 1, wobei
die funktionelle Beschichtungsgruppe (3) eine mehrschichtige, interferenzoptisch variable Beschichtung ist und das optische Fälschungsschutzelement auf einer beliebigen Seite der mehrschichtigen, interferenzoptisch variablen Beschichtung eine interferenzoptisch variable Charakteristik aufweist.

7. Optisches Fälschungsschutzelement gemäß Anspruch 1, wobei
die Reliefstruktur (2) ferner einen dritten Bereich (C) mit einer dritten Mikrostruktur umfasst, wobei ein Tiefe-zu-Breite-Verhältnis der dritten Mikrostruktur größer als ein Tiefe-zu-Breite-Verhältnis der zweiten Mikrostruktur ist und ein spezifisches Volumen der dritten Mikrostruktur größer als ein spezifisches Volumen der ersten Mikrostruktur ist;
die erste Beschichtung (31) und die zweite Beschichtung (33) nicht in dem dritten Bereich (C) angeordnet sind; und das optische Fälschungsschutzelement in dem dritten Bereich (C) eine hohle Charakteristik aufweist.

8. Optisches Fälschungsschutzelement gemäß Anspruch 7, wobei
das Tiefe-zu-Breite-Verhältnis der dritten Mikrostruktur größer als 0,2 und kleiner als 1 ist;
das Tiefe-zu-Breite-Verhältnis der zweiten Mikrostruktur größer als 0 und kleiner als 0,3 ist; und
das spezifische Volumen der dritten Mikrostruktur größer als 0,4 µm³/µm² und kleiner als 3 µm³/µm² ist.

9. Verfahren zur Herstellung eines optischen Fälschungsschutzelements, umfassend:
S1) Bilden einer Reliefstrukturschicht (2), wobei die Reliefstrukturschicht (2) einen ersten Bereich (A) mit einer ersten Mikrostruktur und einen zweiten Bereich (B) mit einer zweiten Mikrostruktur umfasst, wobei ein spezifisches Volumen der zweiten Mikrostruktur größer als ein spezifisches Volumen der ersten Mikrostruktur ist;
S2) Bilden einer ersten Beschichtung, einer dielektrischen Schicht, einer zweiten Beschichtung und einer Schutzschicht, die der Reihe nach gestapelt auf einer Seite der Reliefstrukturschicht (2) angeordnet sind; und
S3) Platzieren eines halb fertiggestellten Produkts bei S2) in eine Atmosphäre, die fähig ist, mit der zweiten Beschichtung zu reagieren, bis ein Teil der oder die gesamte zweite Beschichtung, die in dem zweiten Bereich (B) angeordnet ist, entfernt ist, und wenigstens eine erste Beschichtung (31) und eine zweite Beschichtung (33) nur in dem ersten Bereich gestapelt zurückbleiben, wobei die erste Beschichtung (31) und die zweite Beschichtung (33) nicht-entfernte Teile der ersten Beschichtung und der zweiten Beschichtung sind, die jeweils in dem ersten Bereich (A) angeordnet sind.

10. Verfahren zur Herstellung eines optischen Fälschungsschutzelements gemäß Anspruch 9, wobei
die Reliefstrukturschicht (2) bei S1) ferner einen dritten Bereich (C) mit einer dritten Mikrostruktur umfasst, wobei ein Tiefe-zu-Breite-Verhältnis der dritten Mikrostruktur größer als ein Tiefe-zu-Breite-Verhältnis der zweiten Mikrostruktur ist und ein spezifisches Volumen der dritten Mikrostruktur größer als ein spezifisches Volumen der ersten Mikrostruktur ist.

11. Verfahren zur Herstellung eines optischen Fälschungsschutzelements gemäß Anspruch 10, ferner umfassend:
S4) Platzieren eines halb fertiggestellten Produkts bei S3) in eine Atmosphäre, die fähig ist, mit der ersten und der zweiten Beschichtung zu reagieren, bis ein Teil der oder die gesamte erste Beschichtung und zweite Beschichtung, die in dem zweiten Bereich (C) angeordnet sind, entfernt sind.

12. Verfahren zur Herstellung eines optischen Fälschungsschutzelements gemäß Anspruch 11, wobei
die erste Beschichtung (31) oder die zweite Beschichtung (33) bei S3) eine Aluminiumschicht umfasst oder die erste Beschichtung (31) und die zweite Beschichtung (33) bei S3) eine Aluminiumschicht umfassen; und
eine Säureflüssigkeit oder eine Alkaliflüssigkeit als die Atmosphäre ausgewählt wird, die fähig ist, bei S4) mit der ersten Beschichtung und/oder der zweiten Beschichtung zu reagieren.

13. Verfahren zur Herstellung eines optischen Fälschungsschutzelements gemäß einem der Ansprüche 9-12, ferner umfassend:
Aufbringen einer anorganischen oder organischen Beschichtung oder Anwenden eines Farbschichtverfahrens.

## Revendications

1. Élément anti-contrefaçon optique, comprenant :
une couche à structure en relief (2) ;
la couche à structure en relief (2) comprend une première région (A) ayant une première microstructure et une deuxième région (B) ayant une deuxième microstructure, un volume spécifique de la deuxième microstructure est supérieur à un volume spécifique de la première microstructure ;
un premier revêtement (31), une couche diélectrique (32), un deuxième revêtement (33) et une couche protectrice (4) empilés en séquence sont disposés sur un côté de la couche à structure en relief (2) ;
le premier revêtement (31) et la couche diélectrique (32) sont situés dans la première région (A) et la deuxième région (B), et le deuxième revêtement (33) et la couche protectrice (4) sont situés dans la première région (A), mais ne sont pas situés dans la deuxième région (B) ; et
dans lequel le premier revêtement (31), la couche diélectrique (32) et le deuxième revêtement (33) forment un groupe de revêtement fonctionnel (3), le groupe de revêtement fonctionnel (3) et la première microstructure ont une caractéristique optique combinée dans la première région (A), et le premier revêtement (31) et la deuxième microstructure ont une caractéristique optique combinée dans la deuxième région (B).

2. Élément anti-contrefaçon optique selon la revendication 1, dans lequel
la première microstructure ou la deuxième microstructure est une seule structure ou une structure combinée d'une structure périodique et d'une structure apériodique ; et
une structure en coupe transversale de la première microstructure ou de la deuxième microstructure est n'importe quelle structure ou une structure combinée formée par au moins deux structures quelles qu'elles soient parmi une structure sinusoïdale, une structure de réseau rectangulaire, une structure de réseau trapézoïdal, une structure de réseau blazé et une structure de réseau en forme d'arc.

3. Élément anti-contrefaçon optique selon la revendication 1, dans lequel
le volume spécifique de la première microstructure est supérieur ou égal à 0 µm³/µm² et inférieur à 0,5 µm³/µm² ; et
le volume spécifique de la deuxième microstructure est supérieur à 0,4 µm³/µm² et inférieur à 3 µm³/µm².

4. Élément anti-contrefaçon optique selon la revendication 1, dans lequel
le premier revêtement (31) est relié de façon adjacente à la couche à structure en relief (2).

5. Élément anti-contrefaçon optique selon la revendication 1, dans lequel
un matériau du premier revêtement (31) ou du deuxième revêtement (33) est n'importe quel métal ou un alliage formé par combinaison d'au moins deux métaux quels qu'ils soient parmi le nickel, le chrome, l'aluminium, l'argent, le cuivre, l'étain et le titane ; et
un matériau de la couche diélectrique (32) est n'importe quel composé ou un mélange formé par au moins deux composés quels qu'ils soient parmi le fluorure de magnésium, le dioxyde de silicium, le sulfure de zinc, le nitrure de titane, le dioxyde de titane, le monoxyde de titane, le sesquioxyde de titane, le pentoxyde de trititane, le pentoxyde de tantale, le pentoxyde de niobium, le dioxyde de cérium, le trioxyde de bismuth, le vert d'oxyde de chrome, l'oxyde de fer, l'oxyde d'hafnium et l'oxyde de zinc.

6. Élément anti-contrefaçon optique selon la revendication 1, dans lequel
le groupe de revêtement fonctionnel (3) est un revêtement interférentiel multicouche optiquement variable, et l'élément anti-contrefaçon optique, sur n'importe quel côté du revêtement interférentiel multicouche optiquement variable, a une caractéristique d'interférence optiquement variable.

7. Élément anti-contrefaçon optique selon la revendication 1, dans lequel
la couche à structure en relief (2) comprend en outre une troisième région (C) ayant une troisième microstructure, un rapport profondeur/largeur de la troisième microstructure est supérieur à un rapport profondeur/largeur de la deuxième microstructure, et un volume spécifique de la troisième microstructure est supérieur à un volume spécifique de la première microstructure ;
le premier revêtement (31) et le deuxième revêtement (33) ne sont pas situés dans la troisième région (C) ; et l'élément anti-contrefaçon optique a une caractéristique creuse dans la troisième région (C).

8. Élément anti-contrefaçon optique selon la revendication 7, dans lequel
le rapport profondeur/largeur de la troisième microstructure est supérieur à 0,2 et inférieur à 1 ;
un rapport profondeur/largeur de la deuxième microstructure est supérieur à 0 et inférieur à 0,3 ; et
le volume spécifique de la troisième microstructure est supérieur à 0,4 µm³/µm² et inférieur à 3 µm³/µm².

9. Procédé de fabrication pour un élément anti-contrefaçon optique, comprenant :
51) la formation d'une couche à structure en relief (2), la couche à structure en relief (2) comprend une première région (A) ayant une première microstructure et une deuxième région (B) ayant une deuxième microstructure, un volume spécifique de la deuxième microstructure est supérieur à un volume spécifique de la première microstructure ;
S2) la formation d'un premier revêtement, d'une couche diélectrique, d'un deuxième revêtement et d'une couche protectrice empilés en séquence sur un côté de la couche à structure en relief (2) ; et
S3) la mise en place d'un produit semi-fini en S2) dans une atmosphère pouvant réagir avec le deuxième revêtement jusqu'à ce que tout ou partie du deuxième revêtement situé dans la deuxième région (B) soit retiré, et la conservation au moins d'un premier revêtement (31) et d'un deuxième revêtement (33) empilés uniquement dans la première région (A), dans lequel le premier revêtement (31) et le deuxième revêtement (33) sont des parties non retirées du premier revêtement et du deuxième revêtement qui sont situés dans la première région (A), respectivement.

10. Procédé de fabrication pour un élément anti-contrefaçon optique selon la revendication 9, dans lequel
la couche à structure en relief (2) en S1) comprend en outre une troisième région (C) ayant une troisième microstructure, un rapport profondeur/largeur de la troisième microstructure est supérieur à un rapport profondeur/largeur de la deuxième microstructure, et un volume spécifique de la troisième microstructure est supérieur à un volume spécifique de la première microstructure.

11. Procédé de fabrication pour un élément anti-contrefaçon optique selon la revendication 10, comprenant en outre :
S4) la mise en place d'un produit semi-fini en S3) dans une atmosphère pouvant réagir avec le premier revêtement et le deuxième revêtement jusqu'à ce que tout ou partie du premier revêtement et du deuxième revêtement qui sont situés dans la troisième région (C) soit retiré.

12. Procédé de fabrication pour un élément anti-contrefaçon optique selon la revendication 11, dans lequel
le premier revêtement (31) ou le deuxième revêtement (33) en S3) comprend une couche d'aluminium, ou le premier revêtement (31) et le deuxième revêtement (33) en S3) comprennent une couche d'aluminium ; et
une liqueur acide ou une liqueur alcaline est sélectionnée comme l'atmosphère pouvant réagir avec le premier revêtement et/ou le deuxième revêtement en S4).

13. Procédé de fabrication pour un élément anti-contrefaçon optique selon l'une quelconque des revendications 9 à 12, comprenant en outre :
l'application d'un revêtement inorganique ou organique ou d'un traitement par couche de peinture.
